

# UNITED STATES PATENT OFFICE.

RICHARD ESCALES, OF MUNICH-SCHWABING, GERMANY.

## EXPLOSIVE COMPOUND.

No. 812,195.

Specification of Letters Patent.

Patented Feb. 13, 1906.

Application filed December 31, 1902. Serial No. 187,363.

*To all whom it may concern:*

Be it known that I, RICHARD ESCALES, doctor of philosophy, a subject of the German Emperor, residing at Munich - Schwabing, 5 Germany, (whose post - office address is No. 5 Wilhelmstrasse, Munich-Schwabing, Germany,) have invented certain new and useful Improvements in Explosive Compositions, (for which I have applied for a patent in Germany on the 18th day of November, 1902, in Austria on the 20th day of November, 1902, and in Great Britain on the 20th day of November, 1902,) of which the following is a specification.

15 According to recent researches the disruptive power of explosives may be substantially enhanced by the admixture of finely-divided metals which are easily oxidizable and will consequently get oxidized at the expense of 20 the oxygen contained in the explosive during the deflagration of the latter, which process is accompanied with considerable generation of heat. Further experiments have demonstrated that the physical structure of 25 the metal has much influence on the degree of its action in the explosive composition and that a wooly condition—that is to say, the shape which metals possess in the recently-produced metal wool—is eminently adapted 30 to enhance the dynamic energy or disruptive effect of explosives. These readily-combustible metal wools which, moreover, possess catalytic properties, an extraordinary degree of fineness, and consequently an enormous surface, produce an effect far superior 35 to that obtainable from the same metals when they are in a state of fine division produced by ordinary mechanical disintegration or comminution of the metals in a compact condition. The oxygen or oxygen-carrier forming 40 part of the explosive composition may be in the shape hitherto used for similar purposes.

Among the metals hitherto tested as addition to explosives aluminium (in the shape of aluminium wool) has been found eminently useful. The quantity depends, of course, upon the nature of the explosive and the especial effect desired and may in some cases 45 amount to fifty per cent. of the quantity of

the explosive employed. Hitherto the following three examples have given the best results:

I. Picric acid, eighty parts; aluminium wool, twenty parts.

II. Westfalite, eighty-five parts; aluminium wool, fifteen parts.

III. Carbonite, ninety parts; aluminium wool, ten parts.

The ingredients of Westfalite referred to 60 consists of resin and ammonium nitrate and the ingredients of the carbonite referred to are nitroglycerin, kisselguhr, wood meal, and potassium nitrate.

The great superiority as regards its influence 65 on the dynamic effect of explosives which metal wool possesses in comparison with the fine metallic powers hitherto employed for this purpose may be utilized in the manufacture of explosives, properly speaking, 70 and also in the manufacture of priming compositions for percussion-caps and detonators.

Among the metals which may be used as admixtures in my improved explosive composition are, for instance, magnesium, aluminium, zinc, and iron.

What I claim is—

1. An explosive composition containing an oxygen-carrier and in addition an easily-oxidizable metal in the shape of metal wool for 80 enhancing the dynamic effect of the said composition.

2. An explosive composition containing an oxygen-carrier and in addition aluminium wool for enhancing the dynamic effect of said 85 composition.

3. An explosive composition consisting of Westfalite and aluminium wool, substantially as described.

4. An explosive composition containing 90 ammonium nitrate and aluminium wool, substantially as described.

In witness whereof I have hereunto signed my name in the presence of two subscribing witnesses.

RICHARD ESCALES.

Witnesses:

H. KEINACH,  
C. RATH.